

[54] CORROSION-RESISTANT ALLOYS

[75] Inventor: John H. Culling, Kirkwood, Mo.

[73] Assignee: Carondelet Foundry Company, St. Louis, Mo.

[22] Filed: Sept. 11, 1974

[21] Appl. No.: 505,005

[52] U.S. Cl. .... 75/171

[51] Int. Cl. .... C22c 19/00

[58] Field of Search .... 75/171, 170; 148/32, 32.5

[56] References Cited

UNITED STATES PATENTS

3,759,704 9/1973 Culling..... 75/171

Primary Examiner—R. Dean

Attorney, Agent, or Firm—Koenig, Senniger, Powers  
and Leavitt

57] ABSTRACT

An air-melttable, castable, workable, low hardness

alloy resistant to sulfuric acid over a wide range of acid concentrations. The alloy consists essentially of between 50.18 and about 55.48% by weight nickel, between 33.20 and about 35.15% by weight chromium, between 3.23 and about 3.85% by weight molybdenum, between about 2.85 and about 3.86% by weight copper, up to 1.50% by weight silicon, up to about 2.50% by weight manganese, up to about 1.00% by weight titanium, up to about 1.00% by weight niobium, up to about 1.00% by weight tantalum, up to about 0.01% by weight boron, up to about 0.30% by weight of a rare earth component selected from the group consisting of cerium, lanthanum and misch metal, and carbon in a proportion between 0 and a maximum which is the greater of 0.08% by weight and the sum of  $[Ti/5] + [Nb/8] + [Ta/16]$  where  $[Ti]$  is the titanium content,  $[Nb]$  is the niobium content and  $[Ta]$  is the tantalum content. The sum of the tantalum content and the niobium content is no greater than about 1.00% by weight. The balance of the alloy is essentially iron.

6 Claims, No Drawings

## CORROSION-RESISTANT ALLOYS

## BACKGROUND OF THE INVENTION

This invention relates to corrosion-resistant alloys and, more particularly, to weldable, machinable and workable alloys of low hardness which are resistant to corrosion by both oxidizing and reducing sulfuric acid solutions over a wide range of acid strengths.

Sulfuric acid is an ubiquitous industrial reagent which is generally very corrosive to most metals. The corrosivity of sulfuric acid to any given metal, however, varies widely with the strength of the acid, the temperature of the acid environment, and the nature and concentration of various contaminants. Because of the wide ranging uses for sulfuric acid, industrial process streams may be found which run the gamut of sulfuric acid concentrations; which must be handled from temperatures below room temperature up to the boiling point of the acid; and which contain an extensive variety of contaminants, for example, other acids and salts.

For purposes of analyzing and predicting their corrosive effect on metals, acids and other corrosive agents are commonly classified as either "oxidizing" or "reducing." A reducing medium is generally defined as one which includes no component more oxidizing than the hydrogen ion or hydronium ion while an oxidizing medium is one which does contain such a component. Sulfuric acid, along with such other common materials as hydrochloric acid, acetic acid, phosphoric acid, aluminum chloride, hydrobromic acid, and hydrofluoric acid, is normally a reducing medium. At concentrations above approximately 85% by weight, however, sulfuric acid becomes an oxidizing agent. If its temperature is elevated, sulfuric acid may be oxidizing at even lower concentrations. Thus, a 60% by weight sulfuric acid solution becomes oxidizing at temperatures in excess of 150°F. Even lower concentrations of sulfuric acid can be moderately to strongly oxidizing when they contain various oxidizing acids and salts. Among the most common solutions of this type are the so-called "mixed acids", which are mixtures of sulfuric acid and nitric acid used in organic nitration processes. Other oxidizing materials, some of which may be found in industrial sulfuric acid streams, include hydrogen peroxide, ferric sulfate, silver nitrate, potassium nitrate, sodium nitrate, copper sulfate, potassium permanganate, sodium dichromate, chromic acid, calcium chloride, mercuric chloride, aqua regia, sodium, sodium hypochlorite, ferric chloride, and cupric chloride.

Because of this variety in the character of various industrial sulfuric acid streams, there are relatively few alloys available which can be said to be generally useful in sulfuric acid service. For example, nickel, chromium, molybdenum and copper have all been recognized as useful constituents of alloys designed for exposure to sulfuric acid, yet many combinations of these elements which quite satisfactorily resist the corrosive effect of reducing type sulfuric acid solutions may fail rapidly if a small proportion of an oxidizing agent is present. Other alloys of the same elements may be more resistant to oxidizing media but fail rapidly in a reducing acid. Alloys having other combinations of proportions may be resistant at ambient temperature but fail rapidly at elevated temperatures.

Many alloys which resist dilute sulfuric acid solutions are completely unsuitable for sulfuric acid solutions having concentrations in excess of 60% or 70% by

weight. Many other alloys, in particular those containing 5-23% nickel and 8-18% chromium, demonstrate excellent resistance to sulfuric acid solutions of less than 25% or greater than 80% strength, but fail rapidly in solutions of intermediate concentration. Certain other alloys are available which are highly resistant to a wide range of sulfuric acid solutions, including concentrated sulfuric acid but, for the most part, broadly resistant alloys have been relatively expensive (for example, that sold under the trade designation "Illiium 98" by Stainless Foundry and Engineering Company, Inc.) or have suffered from undesirable mechanical or other properties often due to the presence of large proportions of silicon. Common drawbacks of such alloys have been poor machinability and weldability, with poor workability being an almost universal problem, i.e., few of these alloys can be feasibly produced in wrought form.

The alloys described in my U.S. Pat. No. 3,759,704 provide an important improvement over alloys previously available for sulfuric acid service. The alloys described in that patent are resistant to a wide range of sulfuric acid solution concentrations in both the oxidizing and reducing ranges, and many of the alloys described in that patent may be welded, machined and worked. However, those alloys have relatively high hardnesses in the range of 162-240 Brinell hardness, depending on the exact composition and heat treatment. A continuing need has, therefore, existed for alloys having the superior corrosion properties of those described in U.S. Pat. No. 3,759,704, yet possessing lower hardnesses and correspondingly higher elongations for improved adaptability to welding, machining and working.

## SUMMARY OF THE INVENTION

It is an object of the present invention to provide novel alloys which are resistant to sulfuric acid solutions over a wide range of concentrations. A further object of the present invention is the provision of such alloys which are resistant to sulfuric acid at elevated temperatures. Another object of the present invention is the provision of such alloys which are resistant to sulfuric acid solutions containing oxidizing contaminants. It is a particular object of the present invention to provide such alloys which have a low hardness and are, thus, highly susceptible to welding, machining and working. Other objects and features will be in part apparent and in part pointed out hereinafter.

The present invention is, therefore, directed to an alloy resistant to corrosion by both oxidizing and reducing sulfuric acid solutions over a wide range of acid strengths. The alloy consists essentially of between about 50.18 and about 55.48% by weight nickel, between about 33.20 and about 35.15% by weight chromium, between about 3.23 and about 3.85% by weight molybdenum, between about 2.85 and about 3.86% by weight copper, up to about 1.50% by weight silicon, up to about 2.50% by weight manganese, up to about 1.00% by weight titanium, up to about 1.00% by weight niobium, up to about 1.00% by weight tantalum, up to about 0.01% by weight boron, up to about 0.30% by weight of a rare earth component selected from the group consisting of cerium, lanthanum and misch metal, carbon in a proportion between 0 and a maximum which is the greater of 0.08% by weight and the sum of  $[Ti]/5 + [Nb]/8 + [Ta]/16$  where  $[Ti]$  is the ti-

tanium content, [Nb] is the niobium content, and [Ta] is the tantalum content, and the balance essentially iron. The sum of the tantalum content and the niobium content is no greater than about 1.00% by weight.

### DESCRIPTION OF THE PREFERRED EMBODIMENTS

The alloys of the present invention, like those of U.S. Pat. No. 3,759,704, are highly resistant to corrosion by sulfuric acid solutions over a wide range of compositions. These alloys are resistant to both oxidizing and reducing sulfuric acids and are suitable for use at elevated temperatures. The fabricability properties of the instant alloys, however, are improved over the alloys of U.S. Pat. No. 3,759,704. The alloys of the present invention exhibit substantially lower hardnesses, for example, in the range of 120-130 Brinell Hardness as compared to the alloys of the aforesaid patent which range typically from 160-240 Brinell Hardness. As a consequence, the alloys of this invention exhibit high ductility or tensile elongation and are exceptionally well adapted to all fabricating techniques, including welding, machining, forging and other methods of working.

The essential components of the alloys of this invention are:

|            |              |
|------------|--------------|
| Nickel     | 50.18-55.48% |
| Chromium   | 33.20-35.15% |
| Molybdenum | 3.23-3.85%   |
| Copper     | 2.85-3.86%   |
| Iron       | to make 100% |

The significantly higher nickel content and carefully controlled proportions of chromium, molybdenum and copper impart low hardness values and high tensile elongation or ductility values to these alloys.

Optionally, the alloys of the invention may also include carbon, silicon, manganese, titanium, niobium, tantalum and boron.

attack. The presence of about 0.4 to about 0.6% by weight of either titanium or niobium is, nonetheless, preferred for purposes of enhancing the workability of the alloy.

Further contribution to workability is afforded by very minor proportions of boron up to about 0.01% by weight. Higher proportions of boron should be avoided because of potentially adverse effect on corrosive properties.

Up to about 2.50% by weight manganese and up to about 1.50% by weight silicon may be advantageously included as deoxidizers and aids to castability of the alloys of the invention. For maximum workability and minimum hardness, however, the silicon content is preferably no higher than about 0.75% by weight. Only very low proportions of manganese and silicon are ever necessary in these alloys since molybdenum, copper, chromium and nickel all provide excellent cleanliness and castability in the ranges of proportions above specified. Often the desired proportions of silicon and manganese may be present as impurities in commonly used melting ingredients.

Optionally, cerium, lanthanum or misch metal may be included to enhance workability of the alloys. Up to a total of about 0.30% by weight cerium, lanthanum and/or misch metal may be included.

The alloys of the invention are prepared by conventional methods of melting and no special conditions such as controlled atmospheres or protective slags are required. In preparing the alloys, the constituents of a melting furnace charge need not be of any particular type. Thus, raw materials such as remelt scrap, copper scrap, ferro alloys such as ferromanganese, and other commercial melting alloys may be used.

The following examples illustrate the invention.

### EXAMPLE I

One hundred-pound heats of two different alloys were prepared in accordance with the invention. Each of these heats was then melted in a 100 lb. high fre-

TABLE I

| Alloy No. | PERCENTAGE BY WEIGHT OF ALLOYING ELEMENTS |      |      |       |       |      |      |     |
|-----------|-------------------------------------------|------|------|-------|-------|------|------|-----|
|           | C                                         | Si   | Mn   | Ni    | Cr    | Mo   | Cu   | Fe* |
| 1071      | 0.05                                      | 0.31 | 1.41 | 55.48 | 33.20 | 3.23 | 2.85 | 3.5 |
| 1171      | 0.08                                      | 0.71 | 0.31 | 50.18 | 35.15 | 3.85 | 3.86 | 5.9 |

\*By Difference

Tantalum, titanium and niobium all serve as carbon stabilizers which inhibit the intergranular corrosive attack which may otherwise result from the presence of excessive quantities of carbon. Five parts by weight of titanium stabilizes up to one part by weight carbon, 8 parts by weight niobium stabilizes up to one part by weight carbon, and 16 parts by weight tantalum stabilizes up to one part by weight carbon. Thus, where the maximum proportions of titanium and niobium are present in the alloy, the carbon content may be as high as 0.325% by weight. If the carbon content is maintained at about 0.08% by weight or lower, however, intergranular corrosion can be prevented by proper solution heat treatment and quenching, without the necessity of adding titanium, tantalum or niobium. If the carbon content is about 0.03% by weight or less, moreover, neither heat treatment nor titanium/tantalum/niobium additions are necessary to prevent intergranular

quency induction furnace. The compositions of these alloys are set forth in Table I.

Two standard physical test blocks and three corrosion test bars were prepared from each heat. One of the physical test blocks from each alloy was solution annealed at 1,950°F for 3 hours and then oil quenched. The physical properties of these alloys as measured in the as-cast state are set forth in Table II.

TABLE II

| Alloy No. | Tensile Strength PSI | Yield Strength PSI | Percent Elongation | Brinell Hardness |
|-----------|----------------------|--------------------|--------------------|------------------|
| 1071      | 61,210               | 34,400             | 46.4               | 121              |
| 1171      | 62,050               | 36,500             | 30.5               | 128              |

The corrosion test bars were also annealed for 30 minutes at 1,950°F. and oil quenched prior to machin-

ing into 1 1/2 inch diameter by one-fourth inch high discs having a one-eighth inch diameter hole in the center. Twelve to 14 discs were obtained for each alloy.

These discs were used in the comparative corrosion tests described hereinafter comparing the performance of the alloys of the invention with two prominent commercially available alloys. The compositions of the commercially available alloys which were used in these tests, their physical properties in the as-cast state, and the respective trade designations under which they are marketed are set forth in Table III.

mula in accordance with ASTM specification G1-67.

$$R_{ipy} = 0.3937 \frac{W_o - W_f}{ADT} \quad \text{where}$$

$R_{ipy}$  = corrosion rate in inches per year

$W_o$  = original weight of sample

$W_f$  = final weight of sample

$A$  = area of sample in square centimeters

$T$  = duration of test in years

$D$  = density of alloy in g./cc.

Results of this corrosion test are set forth in Table IV.

TABLE III

COMPOSITION AND PHYSICAL PROPERTIES OF  
COMMERCIALLY AVAILABLE ALLOYS IN AS CAST STATE

| Alloy Name      | C%   | Si%  | Mn%  | Ni%  | Cr%  | Mo% | Cu% | Fe%* | Tensile Strength<br>PSI | Yield Strength<br>PSI | Percent<br>Elongation | Brinell<br>Hardness |
|-----------------|------|------|------|------|------|-----|-----|------|-------------------------|-----------------------|-----------------------|---------------------|
| Illium 98       | 0.05 | 0.79 | 1.25 | 55.0 | 28.0 | 8.5 | 5.5 | 1    | 54,000                  | 41,000                | 18.0                  | 160                 |
| Carpenter 20Cb3 | 0.05 | 0.70 | 1.40 | 34.0 | 20.0 | 2.5 | 3.5 | 37   | 69,000                  | 31,500                | 36.0                  | 155                 |

\*By Difference

TABLE IV

CORROSION RATES AS LOSSES IN INCHES OF PENETRATION PER  
YEAR FOR VARIOUS SULFURIC ACID-WATER SOLUTIONS AT 80°C.

| Alloy No.<br>or Name | 10%<br>$H_2SO_4$ | 25%<br>$H_2SO_4$ | 40%<br>$H_2SO_4$ | 50%<br>$H_2SO_4$ | 60%<br>$H_2SO_4$ | 70%<br>$H_2SO_4$ | 93%<br>$H_2SO_4$ | 96%<br>$H_2SO_4$ |
|----------------------|------------------|------------------|------------------|------------------|------------------|------------------|------------------|------------------|
| 1071                 | 0.0027           | 0.0030           | 0.0043           | 0.0019           | 0.0005           | 0.0008           | 0.0040           | 0.0019           |
| 1171                 | 0.0022           | 0.0032           | 0.0030           | 0.0016           | 0.0003           | 0.0068           | 0.0038           | 0.0013           |
| Illium 98            | 0.0030           | 0.0057           | 0.0048           | 0.0050           | 0.0044           | 0.0107           | 0.0040           | 0.0033           |
| Carpenter<br>20Cb3   | 0.0041           | 0.0102           | 0.0091           | 0.0083           | 0.0102           | 0.0512           | 0.0202           | 0.0173           |

## EXAMPLE 2

Comparative corrosion tests were run in 10%, 25%, 40%, 50%, 60%, 70%, 93% and 96% sulfuric acid solutions at 80°C.

Disc samples of Illium 98 and Carpenter 20Cb3 were prepared having the same dimensions as the discs prepared in Example 1. Residual machining oil and dirt were removed from all of the sample discs by cleaning with a small amount of carbon tetrachloride. The discs were then rinsed in water and dried. Each disc was weighed to the nearest ten-thousandth of a gram and then suspended in a beaker by a piece of thin platinum wire hooked through the center hole of the disc and attached to a glass rod which rested on the top of the beaker. Sufficient sulfuric acid solution was then added to the beaker so that the entire sample was surrounded. The temperature of the acid was thermostatically controlled at 80°C. by means of a water bath and each beaker was covered with a watch glass to minimize evaporation.

After precisely six hours, the sample discs were removed from the sulfuric acid solution and cleaned of corrosion products. Most samples were cleaned sufficiently with a small nylon bristle brush and tap water. Those samples on which the corrosion product was too heavy for removal with a nylon brush were cleaned with a one-to-one solution of hydrochloric acid and water. After the corrosion products had been removed, each disc was again weighed to the nearest ten-thousandth of a gram. The corrosion rate of each disc, in inches per year, was calculated by the following for-

In view of the above, it will be seen that the several objects of the invention are achieved and other advantageous results attained.

As various changes could be made in the above products without departing from the scope of the invention, it is intended that all matter contained in the above description shall be interpreted as illustrative and not in a limiting sense.

What is claimed is:

1. An air-meltable, castable, workable low hardness alloy resistant to corrosion by sulfuric acid over a wide range of acid concentrations consisting essentially of between about 50.18 and about 55.48% by weight 50 nickel, between about 33.20 and about 35.15% by weight chromium, between about 3.23 and about 3.85% by weight molybdenum, between about 2.85 and about 3.86% by weight copper, up to about 1.50% by weight silicon, up to about 2.50% by weight manganese, up to about 1.00% by weight titanium, up to about 1.00% by weight niobium, up to about 1.00% by weight tantalum, up to about 0.01% by weight boron, up to about 0.30% by weight of a rare earth component selected from the group consisting of cerium, lanthanum and misch metal, carbon in a proportion between 0 and a maximum which is the greater of 0.08% by weight and the sum of

$$\frac{[Ti]}{5} + \frac{[Nb]}{8} + \frac{[Ta]}{16}$$

where

[Ti] = the titanium content

[Nb] = the niobium content

[Ta] = tantalum content

the sum of the tantalum content and the niobium content being no greater than about 1.00% by weight, and the balance essentially iron.

2. An alloy as set forth in claim 1 having a titanium content of between about 0.4 and about 0.6% by weight.

3. An alloy as set forth in claim 1 having a niobium content of between about 0.4 and about 0.6% by weight.

4. An alloy as set forth in claim 1 having a silicon content no greater than about 0.75% by weight.

5. An alloy as set forth in claim 1 comprising approximately 55.48% by weight nickel, approximately

33.20% by weight chromium, approximately 3.23% by weight molybdenum, approximately 2.85% by weight copper, approximately 0.31% by weight silicon, approximately 1.41% by weight manganese, approximately 0.05% carbon and approximately 3.5% by weight iron.

6. An alloy as set forth in claim 1 comprising approximately 50.18% by weight nickel, approximately 35.15% by weight chromium, approximately 3.85% by weight molybdenum, approximately 3.86% by weight copper, approximately 0.71% by weight silicon, approximately 0.31% by weight manganese, approximately 0.08% by weight carbon and approximately 5.9% by weight iron.

\* \* \* \* \*

20

25

30

35

40

45

50

55

60

65